

Nov. 20, 1951

G. J. SLUITER

2,575,895

METHOD OF MAKING FIBROUS PRODUCTS

Filed Sept. 22, 1949



FIG.1



FIG.5



FIG.2



FIG.6



FIG.3



FIG.7



FIG.4



FIG.8

INVENTOR:  
GERRIT JOHANNES  
SLUITER  
By *Robert E. Burns*  
ATTORNEY

## UNITED STATES PATENT OFFICE

2,575,895

## METHOD OF MAKING FIBROUS PRODUCTS

Gerrit Johannes Sluiter, Amsterdam, Netherlands

Application September 22, 1949, Serial No. 117,247  
In the Netherlands September 30, 1948

5. Claims. (Cl. 260—742)

1

The invention relates to a process for the preparation of a fibrous pap for the manufacture of artificial products and in particular to a process for the preparation of a uniform pap, substantially consisting of fibrous material, glue and rubber latex.

It is known that in opening in water fibre aggregates such as chemically free cellulose in a more or less pure condition in the form of pulp or wadding of wood, straw or the like, it is very difficult to disengage the fibres from each other. In rubbing a sample between the fingers the fibres stick together in the form of barley-corn-like clods. This phenomenon interferes in different processes in which fibres are worked up into uniform artificial masses.

The present invention has in view to meet this objection in making firstly a uniform fibrous suspension by that dry fibre aggregates are added to, mixed with and exposed to the action of a uniform aqueous glue dispersion and thereupon thoroughly beaten through this glue dispersion before the whole is worked up with aids and appliances into a uniform fibrous pap from which the artificial products are to be manufactured.

It is found that by application of this process a much better uniform distribution of the fibres through the pap, from which the artificial products are to be manufactured, is obtained and that in this way the convertibility of the pap and the properties of the artificial products therefrom are improved to an unprecedented extent.

Preferably the fibrous suspension is left to itself for a period of the order of several hours, for example during a day, before the fibres are beaten through the glue dispersion.

In the process according to the invention chemically free cellulose in a more or less pure condition in the form of pulp or wadding of wood, straw, or the like can advantageously be used as a fibre aggregate.

It is known per se to work up fibres together with glue and latex and if desired fillers. In the known process the glue was not used, however, for prior preparation of a uniform fibrous glue suspension in the above indicated way. Also the glue was added irrespectively of whether fibrous fillers were used or not, and naturally the applied percentage of glue was not specifically adapted to the applied amount of fibrous material.

In the process according to the invention the glue can be of vegetable origin, such as vegetable protein glue, starch products from gluten (zeine), starch derivative agglutinants (dextrin, swelled

2

starch), cellulose derivative agglutinants such as tylose (methyl cellulose), gums and resins (such as gum tragacanth) included, as well as of animal origin such as the meat-, fish- and bone-glues and the casein- and albumin-glues, and also of synthetic origin.

In selecting the glue, it has to be considered that it is undesirable in several cases that the products give out unpleasant smells. In particular with proteinous glue these may assert themselves in an awkward degree in exposing to the air.

The minimum amount of glue that is necessary is determined by the requirement that a sufficient disengagement of the fibres and a uniform distribution throughout the glue dispersion is obtained.

The invention will be more fully understood from the following detailed description in conjunction with the accompanying drawings in which:

Figs. 1 to 8 are fragmentary perspective views of coverings made in accordance with the invention.

25 Without restricting the invention to the recipe following hereafter, an example for the preparation of a uniform suspension of fibres in aqueous glue is now given. Naturally the process for the preparation of the glue dispersion used therein depends on the character of the glue and therefore is liable to alterations.

## Example 1

35 5-25 parts by weight of glue, for example the Swedish natural starch product known under the registered trade-mark "Alkasit," is stirred 1:10 with water. The mass is thoroughly mixed and then preferably left for swelling during some time, for example  $\frac{1}{2}$ -1 hour. The thus obtained thick uniform paste is diluted with water, 1:1. Into the ready glue dispersion fibre aggregate is introduced in one or more charges, for example 75 parts by weight of cellulose, e. g. wadding, made from chemical pulp used in the manufacture of paper, thereupon mixed with the glue dispersion and left standing for some time, for example during a day. Thereupon the fibres are thoroughly beaten through the glue dispersion until a uniform pap is obtained.

40 45 50 55 The thus obtained fibrous suspension can advantageously be applied for mixing with rubber latex. Whereas it is extremely difficult to mix dry fibres such as cellulose with latex without coagulation unless the latex is stabilized very thoroughly, fibrous suspensions obtained accord-

ing to the process of the invention are very uniform and mixable without coagulation with normally preserved, inhibited and stabilized latex.

Preferably cream latex, that is latex which is concentrated to about 60 percent by weight of solids, is used therein. It is true that the so called "revertex," which is concentrated to amply 70 percent by weight of solids, may also be used, but usually it is too expensive. Latices containing more water, such as latex with about 38-40 percent by weight of solids will give a pap that is too thin for some objects if the ratio of solids in the pap is wanted to be maintained. Natural rubber latex as well as synthetic latices can be used. The latices may contain self vulcanizing agents and accelerators.

As a greater ratio of rubber is incorporated in the pap, the products obtained from the latter will be of better quality; the higher latex contents and the higher concentrations of fibres and aids and appliances coupled therewith simultaneously increase the cost price however.

To illustrate this application of the fibrous suspensions the following recipe is given:

*Example 1'*

125 parts by weight of cream latex containing stabilizer, anti-oxidant and preservator is added under stirring to the pap obtained accordingly to the preceding Example 1.

By making use of the above mentioned principle it is possible, if desired under addition of aids and appliances, to prepare a pap which, according to the composition, can be worked up by brushing up, bulking, casting, spraying and the like to a covering material for walls, ceilings, floors, walls and seats of furniture, trunks, human bodies and the like. In that case the pap can be superposed either onto the surface that is to be covered or firstly onto a supporting layer of paper, board, fabric and the like, which layer may or may not be removed after drying. Prior to the drying, relief may be pressed into the superposed pap if desired.

A plurality of coverings made in accordance with the invention are shown by way of example in the drawings. Fig. 1 shows a covering consisting of a layer 1 made from the final pap only and thus substantially consisting of rubber, fibres, glue, aids and appliances. Fig. 2 shows a covering consisting of a layer 1 superposed on a supporting underlayer 2. Fig. 3 shows a covering consisting of two layers 1 with an intermediate supporting layer 3. Fig. 4 illustrates the removal of the underlayer 2 from the layer 1 of the covering shown in Fig. 2. Figs. 5 to 8 correspond to Figs. 1 to 4 respectively and show the coverings thereof provided with a relief 4.

Fillers may be added to increase the hardness of the products manufactured with the pap. Very suitable for this purpose is, for example chalk, of which according to the desired increase of the hardness, more or less is added (for example 125-300 parts by weight), mixed with water in a ratio that is dependent i. e. on the filler quality. Thus it makes a difference e. g. whether the chalk is medicinal or twice washed. The ratio lies mostly at about 1:1. The most uniform distribution is obtained by adding these fillers to the glue dispersion, i. e. prior to the addition of the fibre mass.

Still harder products can be obtained by incorporation of gyps (plaster), cement or similar fast-hardening materials, for example 100 parts by weight in 50 parts of water. These ingredients

may be added to the glue dispersion or to one of the subsequent semimanufactured products or to the final product.

In order to increase the cohesion capacity on surfaces (walls and the like), to increase the mechanical strength and to decrease the stickiness of the products to be manufactured, water glass is generally added, for example 30 parts by weight in 60-70 parts of water. This may be done during the beating of the fibres through the glue dispersion, or the water glass may be added later on, even simultaneously with the addition of the latex.

Pigments may be added to any of the components of the pap, or to the semi-manufactured or final product. Preferably latex dye is used for this purpose as only a small quantity thereof is necessary thanks to its strong colouring power.

In some cases application of latex with self vulcanizers and accelerators is of special advantage, for example if covering material for furniture has to be manufactured or if the pap is worked together with an under or intermediate layer of fabric.

Though the products obtained from the pap are poorly inflammable, it can be useful in special cases, such as for wall coverings in ships, theatres and the like to decrease the inflammability by addition of powdered asbestos, alum and the like, preferably to the fibrous material prior to the addition of the latter to the glue dispersion.

Mention has already been made of the fact that the pap can be made as a sprayable pap. For that purpose it is necessary that the water ratio is higher than for the spreadable pap. A satisfactorily sprayable product can be obtained for example by addition of a suitable amount of water to the spreadable pap or by addition of this extra water during one or more steps of the preparation of the pap.

Another suitable sprayable pap can be obtained according to the following example.

*Example 1''*

To 100 parts by weight of a solution of caseinate glue and borax in water in a ratio by weight of 10:4:80 a preservator is admixed. Half of this bath is added to 167 parts by weight of cream latex together with vulcanisation dispersion. The remaining half is added to the pap obtained according to Example 1, during the preparation of which 200 parts by weight of chalk in 400 parts of water and 30 parts by weight of water glass in 70 parts of water are added. Thereupon the latex liquid and the pap are mixed under stirring.

In preparing a sprayable pap it is recommended to add a frother such as a special soap. The spraying can be carried out i. e. with the aid of a special motar gun with compressor.

A particular property of very great importance for products that are manufactured with latex, is the porosity. By application of the fibrous suspension obtained by the process according to the invention it appears that a rubber cellulose product can be manufactured that is waterproof and nevertheless gas-permeable so that no inconvenience is met with by condensation deposits on the surfaces of these products.

I claim:

1. A process for preparing a fibrous composition containing cellulose fibres, glue and a rubber in aqueous dispersed form which comprises adding 70-80 parts by weight of loosely

cohering fibrous cellulose flock to a uniform aqueous dispersion of 5-25 parts by weight of glue, intimately mixing said fibrous cellulose flock with said glue dispersion, allowing said mixture of cellulose flock and glue dispersion to stand for a period of several hours, thereafter beating the fiber glue dispersion to effect uniform suspension of loose fibers in the glue dispersion, and mixing said suspension with 75-100 parts by weight of rubber solids in latex form, whereby to form a uniform composition adapted to be shaped and dried to form flexible articles.

2. A process as defined in claim 1, wherein an aqueous suspension of 125-300 parts by weight of chalk is added to the glue dispersion prior to the addition of the cellulose flock.

3. A process as defined in claim 1, wherein 20-40 parts by weight of water glass are added to the suspension of loose cellulose fibers in the aqueous glue dispersion after the beating step.

4. A uniform fibrous composition comprising, in intimate admixture, 75-100 parts of a rubber in the form of a latex and an aqueous glue dispersion containing 5-25 parts by weight of glue, and 70-80 parts by weight of loose cellulose fibers suspended therein, said loose cellulose fibers being derived from cellulose flock.

5. A flexible product obtained by removing water from a uniform fibrous composition comprising, in intimate admixture, 75-100 parts of a rubber in the form of a latex and an aqueous glue dispersion containing 5-25 parts by weight of glue, and 70-80 parts by weight of loose cellulose fibers suspended therein, said loose cellulose fibers being derived from cellulose flock.

10

GERRIT JOHANNES SLUITER.

## REFERENCES CITED

The following references are of record in the file of this patent:

## UNITED STATES PATENTS

| Number     | Name            | Date           |
|------------|-----------------|----------------|
| Re. 21,575 | Tator           | Sept. 17, 1940 |
| 1,765,015  | Hopkinson       | June 17, 1930  |
| 1,883,106  | Thoma           | Oct. 18, 1932  |
| 2,127,298  | Isaacs          | Aug. 16, 1938  |
| 2,215,553  | Johnson         | Sept. 24, 1940 |
| 2,278,943  | Oesterreich     | Apr. 7, 1942   |
| 2,333,265  | McIntosh et al. | Nov. 2, 1943   |
| 2,474,801  | Owen            | June 28, 1949  |